

# UNITED STATES PATENT OFFICE.

KARL MARX, OF DESSAU, GERMANY, ASSIGNOR TO ACTIEN GESELLSCHAFT FÜR ANILIN FABRIKATION, OF BERLIN, GERMANY.

## PROCESS FOR DYEING SKINS, HAIRS, AND THE LIKE.

1,183,748.

Specification of Letters Patent. Patented May 16, 1916.

No Drawing.

Application filed July 16, 1914. Serial No. 851,428.

To all whom it may concern:

Be it known that I, KARL MARX, a subject of the Duke of Brunswick, residing at Dessau, Germany, my post-office address being Albrechtstrasse 16, Dessau, Germany, have invented certain new and useful Improvements in Processes for Dyeing Skins, Hairs, and the like, of which the following is a specification.

10 I have found that a series of derivatives of dialkylaminodiphenylamin of the general formula:



in which R means an alkyl group and R<sub>1</sub> signifies a univalent substituent, such as NH<sub>2</sub>, N(CH<sub>3</sub>)<sub>2</sub>, N(C<sub>2</sub>H<sub>5</sub>)<sub>2</sub>, OH or the like, 20 or a suitable derivative of these bodies, are excellently fitted for dyeing skins, hairs and the like. There are thus obtained, generally speaking, gray tints which are fast to weather and storage; the skins to be dyed 25 can be previously mordanted or not. The dyeing operation itself may be performed as usual but without adding an alkaline substance.

The following example illustrates my invention; the parts are by weight: The skin to be dyed is washed for about an hour in water containing 10-20 grams of calcined sodium carbonate per liter, well rinsed and then dyed in a bath which contains per liter 35 3 grams of the hydrochlorid of para-dimethylamino-para'-aminodiphenylamin and about 60 grams of hydrogen peroxid of about 3 per cent. strength. Dyeing is continued for about 3 hours at ordinary temperature with periodical handling. Thereupon 40 the skin is rinsed, submitted to centrifugal action, the flesh side of the skin coated with an emulsion of common salt solution and yolk of egg, and the skin then dried and 45 cleaned. There is obtained a very beautiful greenish-gray which withstands very well the influence of the weather.

On skins mordanted with chromium, quite similar tints are obtained, whereas on 50 skins previously mordanted with iron or

aluminum mordants there are obtained beautiful tints, more blue-gray.

It is obvious that my invention is not limited to the foregoing example or to the details given therein. For instance by dyeing non-mordanted skins in the prescribed manner with para-para'-tetramethyldiaminodiphenylamin hydrochlorid there is obtained a beautiful green-gray tint which also withstands very well the influence of the 55 weather. On a chromium mordant a quite similar tint is obtained.

In like manner by means of para-dimethylamino - para' - oxydiphenylamin a beautiful neutral gray may be produced on 60 non-mordanted skins, which is also fast to weather. On iron and aluminium mordants like tints are produced.

Having now described my invention and the manner in which it may be performed 70 what I claim is,—

1. The herein described process which consists in dyeing skins in the presence of an oxidizing agent not giving rise to an alkaline reaction in a bath which contains a salt 75 of a base of the general formula as follows:



in which R represents an alkyl group and R<sub>1</sub> signifies a univalent substituent.

2. The herein described process which consists in dyeing skins in the presence of hydrogen-peroxid in a bath which contains a salt of a base of the general formula:



in which R<sub>1</sub> signifies a univalent substituent.

3. The herein described process which consists in dyeing skins in the presence of hydrogen-peroxid in a bath which contains a salt of a base of the general formula as follows:



in which R<sub>1</sub> signifies a univalent inorganic substituent.

95

90

85

95

100

4. The herein described process which  
consists in dyeing skins in the presence of  
hydrogen-peroxid in a bath which contains  
a salt of para-dimethylamino-para'-amino-  
5 diphenylamin.

In testimony whereof I have hereunto set

my hand in presence of two subscribing wit-  
nesses.

KARL MARX.

Witnesses:

RUDOLPH FRICKE,  
ALICE DUNGER.